

July 3, 1934.

F. W. HUMPHNER

1,965,289

DECALCOMANIA TRANSFER PAPER

Filed April 24, 1933

*Fig 1.*



*Fig 2.*



*Inventor:*

*Ferdinand W. Humphner,  
By Drydenforth, See, Britton, & Wiles,  
Atty.*

## UNITED STATES PATENT OFFICE

1,965,289

## DECALCOMANIA TRANSFER PAPER

Ferdinand W. Humphner, Oak Park, Ill., assignor  
to Mid-States Gummed Paper Co., Chicago, Ill.,  
a corporation of Illinois

Application April 24, 1933, Serial No. 667,737

2 Claims. (Cl. 41—33)

This invention relates to decalcomania transfer paper and more particularly to a type of decalcomania transfer in which the transfer, after the paper base is moistened, is slipped off the paper and the bottom side of the transfer applied to the new surface.

An object of the invention is to provide a permanently flat or non-curling transfer paper upon which the final prints may be formed. Other specific objects and advantages will appear as the specification proceeds.

The invention is illustrated, in its preferred embodiment, by the accompanying drawing, in which—

15 Figure 1 is a perspective view of a transfer paper embodying my invention, the lacquer and adhesive layers being partially rolled; and Fig. 2, a plan view of the transfer paper, a portion of the lacquer and adhesive layers being torn away.

20 The paper employed may be of any suitable type, a slack sized paper being preferred. To the top side of the paper, I apply a single coating of gum or adhesive, consisting mainly of a blend of animal and vegetable glues. For example, a mixture consisting of 25% of animal glue and 75% of dextrine, may be mixed with equal parts of water and to this may be added 1% of glycerine and 2% of glucose. While this composition has been found satisfactory, it is recognized that the proportions and the constituents may be varied 25 according to the type of adhesive desired. The above mass is mixed thoroughly and then applied to the paper in one coating. The thickness of the mixture is preferably such as to permit the adhesive to flow to a flat level surface without 30 mechanical aid. However, if desired, mechanical means may be employed to form the adhesive layer on the paper.

35 After the adhesive is dry, I prefer to process the paper in a suitable non-curling machine or other apparatus in order to break up the gum layer into a multitude of segments substantially uniformly distributed through the adhesive layer.

40 In view of the fact that the construction of non-curling machines is well known, a detailed description of the mechanism is unnecessary. Ordinarily, the paper is drawn over a breaker bar positioned at an angle of 45° with respect to the paper and then reversed over a second bar at 45° to form a diamond effect on the adhesive coating. In fact, it is only necessary to break or crack 45 the surface of the adhesive and the paper may, if desired, be passed over one edge at right angles 50 to the grain of the paper, causing the adhesive

layer to crack and provide a substantially uniform degree of cracking throughout the layer.

55 After the adhesive surface has been broken up with intersecting cracks throughout the layer, I next cover the adhesive with a layer of lacquer, 60 the constitution of the lacquer being such as to enable it to penetrate the interstices and fill up the voids of the cracks. Also, I prefer to employ a lacquer which is sufficiently tenacious or tough to prevent the cracks from again closing under 65 the various conditions to which the paper may be subjected. There is a tendency for gummed paper, which has been processed in a non-curling machine, to acquire under certain conditions of 70 humidity or temperature, etc., a tendency to again roll or curl. With my transfer paper, the lacquer layer forms a wedge between each of the minute cracks and renders the paper permanently non-curling.

75 The lacquer layer has an affinity for ink so that upon the top of the layer, prints of various forms may be made. For example, printing for tax stamps, etc. may be formed on the top of the lacquer layer.

80 A lacquer of any suitable composition having the desired qualities of sufficient fluidity to penetrate the interstices, sufficient body or toughness, affinity for inks, etc. may be employed. Lacquers having these qualities are well known and a detailed description is unnecessary. Cellulose 85 lacquers having gum constituents and suitable solvents have been satisfactorily employed. By way of example, the following constituents and proportions of a satisfactory lacquer may be stated:

|                    | Parts |
|--------------------|-------|
| Nitrocellulose     | 12    |
| Dibutyl phthalate  | 7     |
| Resin (dammar gum) | 6     |
| Ethyl acetate      | 10    |
| Butyl acetate      | 20    |
| Ethyl alcohol      | 10    |
| Toluol             | 35    |

85 The above proportions are by volume and the composition contains approximately 25% solids.

90 After the transfer paper has been formed, as described above, and the final prints formed on the lacquer top surface, the individual decalcomania transfers may be removed from the paper by first moistening the paper base and then slipping the individual transfers off the paper and applying the bottom side of the transfer to the new surface. The adhesive which secured the lacquer layer to the paper now serves as means 105

110 to the grain of the paper, causing the adhesive

for bonding the transfer to the new surface. The transfer sticks tenaciously to cellophane and the like.

5 In the description above given, the lacquer covers the sheet or strip of paper and the individual or separate prints are formed on the sheet. If desired, the sheet may be perforated between the prints so that the separate transfers may be torn apart with their respective paper bases attached thereto.

10 While I have described adhesive layers and lacquer layers of certain specific compositions, it will be understood that any suitable adhesive or lacquer for the purposes described may be employed. Also, in the processing of the paper, 15 any suitable means for cracking the paper so as to distribute the cracks rather uniformly over the adhesive surface may be used. The foregoing detailed description has been given for 20 clearness of understanding only, and no unne-

cessary limitations should be understood therefrom, but the appended claims should be construed as broadly as permissible, in view of the prior art.

I claim:

1. A decalcomania transfer comprising a paper base, a dry adhesive layer thereon, said adhesive layer having cracks therein and substantially uniformly distributed therethrough, a tough lacquer body over said adhesive and extending between said cracks, and a final print on the top of said lacquer.

2. A decalcomania transfer comprising a paper base, a dry adhesive layer having cracks therein and substantially uniformly distributed therethrough, lacquer extending over said layer of adhesive and between said cracks and having sufficient body to prevent the closing of said cracks, and a final print on the top of said layer.

FERDINAND W. HUMPHNER.

25

102

30

105

35

110

40

115

45

120

50

125

55

130

60

135

65

140

70

145

75

150